

March 29, 1938.

C. B. CHATFIELD

2,112,762

MARKING BOARD AND CRAYON THEREFOR

Filed Jan. 13, 1937

*FIG. 1.*



*FIG. 2.*



INVENTOR

CHARLES B. CHATFIELD.

BY

Ward, Clegg & Neal

ATTORNEYS

## UNITED STATES PATENT OFFICE

2,112,762

## MARKING BOARD AND CRAYON THEREFOR

Charles B. Chatfield, Chicago Heights, Ill.

Application January 13, 1937, Serial No. 120,450

18 Claims.

(Cl. 35—66)

This invention relates to a marking board which may replace the customary blackboard and a crayon for use thereon.

Blackboards, whether of slate or of composition, used with chalk crayons have well-known disadvantages. They must have abrasive surfaces. In the case of the slate the surface is naturally abrasive and under the microscope shows pits with jagged edges covering the entire surface. In the case of artificial or composition blackboards, abrasive such as slate, emery or corundum powder are added to the surface composition to give the necessary jagged edges which project from the surface of the composition board. These abrasive surfaces must be present in these boards in order to scrape off and hold particles of the chalk crayon which has little, if any, adhesiveness for the blackboard surface, but upon being scraped off by these minute abrading surfaces fills the pits or spaces between the abrading edges to give the appearance of a continuous mark. The weak, friable nature of the chalk causes it to dust during writing, for only a portion of the chalk that is abraded from the chalk crayon adheres to the board and the rest of it flies in the air or adheres to the fingers or the clothing. The written or other marks on blackboards are customarily erased with a dry eraser which causes worse dusting than the process of writing for much of the chalk removed by the eraser does not remain on it but flies in the air. The chalk dust so released is a nuisance and may be a menace to health. In addition, the legibility of white or other color on a black background is not as high as certain colors on white or light backgrounds. The scale of legibility appears to be somewhat as follows:—black on yellow, green on white, blue on white, all of which are more legible than any marks on a black background. In addition blackboards after constant use assume a grayish cast which makes writing thereon with white chalk even less legible. In addition to these disadvantages, blackboards absorb considerable light so that a wall lined therewith reflects into a room a correspondingly smaller amount of light.

It is important in using the usual blackboards, as mentioned above, to provide a chalk crayon. These crayons are for the most part composed of natural or artificial mineral substances, such as calcium carbonate, clay, gypsum, plaster of Paris, talc and the like to which pigments are sometimes added to give a desired color. The crayons are made up by compression with or without binders, or cast in molds as in the case

of plaster of Paris. As so prepared because of their friable character they may be used for writing on the abrasive blackboards as mentioned above. Crayons which are not friable and which would overcome the objectionable dusting mentioned above, are not feasible for writing on abrasive blackboards because they tend to fill up the pits or abrading surfaces and cannot be removed or would be removed with difficulty by the usual felt erasers.

The principal object of the present invention accordingly is to provide a writing structure and crayon which shall do away at least to some extent with the mentioned disadvantages of the combined blackboard and chalk crayon, and particularly to provide a board and crayon which shall be substantially free from dusting and which shall produce writing or other marks of a more legible character than heretofore obtainable on blackboards and which shall permit easy repeated marking and erasure and which shall give improved light reflecting characteristics. Another object is to provide a board or similar structure and crayon having the desired characteristics and which may be easily and inexpensively manufactured. Other objects and advantages will more clearly appear in the detailed description hereinafter set forth.

The invention accordingly comprises the novel devices and products and combinations thereof, specific embodiments of which are described hereinafter by way of example and in accordance with which I now prefer to practice the invention.

In the accompanying drawing, which is made part of the specification, I show embodiments of the invention as I now prefer to practice it. In the drawing—

Fig. 1 shows a panel board made up of cement-asbestos board or wood fiber board, etc., on which is a coating of vinylite or other resin containing pigment, on which panel board a crayon containing triethanolamine soap and pigment or like material is employed;

Fig. 2 shows another type of panel board composed of wood fiber board or chip board or other paste-board etc., on which is a laminated sheet of opaque white, yellow or other colored litho-paper, over which is another lamination of clear vinylite or other lacquer or a sheet of cellulose acetate or other cellophane.

I have found in accordance with my invention that the above objects, among others may be accomplished by the combination of a panel drawing board, which is opaque or nearly opaque, hav-

ing a glazed surface of a non-abrasive character substantially without roughnesses except for possible slight undulations, and an unctuous crayon of a color contrasting with that of the board for marking thereon, which crayon when of the size of the usual hand crayon, may be of a toughness so that it will not break if dropped from a height of about four feet, and whose marking surface is tacky when applied to the glazed surface mentioned, which crayon does not soften or harden appreciably at temperatures in a range of 15° F. above or below room temperature, the combination being such that the crayon will deposit on said surface clearly legible marks with about the same drag as that of a soft lead pencil if applied to ordinary writing paper, but which may be removed by simple rubbing without abrasion, such as occurs in erasure of lead pencil marks from paper, with a soft cloth, for example soft cotton, wool or paper (such as Kleenex), without appreciable smearing or stain left on said surface. The board and crayon combination is adapted for repeated marking and erasure without losing the characteristics mentioned.

25 In the appended claims where the expression "panel drawing board" is used, I refer to a panel board attached to a wall replacing the ordinary blackboard for marking, drawing, etc., as well as a smaller type of structure mounted or unmounted and serving to replace the ordinary small blackboard or writing slate.

The usual hand crayon size, which I have referred to in the appended claims, is of approximately  $\frac{1}{4}$  inch diameter and 3 to 4 inches long. It is to be understood that the crayons of my invention are not restricted to such size but may be of any practical size. Hand size crayons heretofore known to me are required to be encased in paper or otherwise. My crayons in such size, however, are sufficiently strong in themselves so that they may be used unencased for hand marking.

I prefer to employ a panel drawing board of opaque or nearly opaque material comprising a relatively flat foundation and a smooth glazed coating adhering to the face of the foundation, the foundation and coating being sufficiently stiff inherently to permit marking by a crayon thereon. The foundation may be of cellulose-containing material such as pasteboard or the like, or cement or sheet metal, molding resin or like material. The coating is preferably of vinylite or cellulose ester, casein or like material either in sheet form or applied as a lacquer. The crayons preferably contain hardening, lubricating and tacky materials and are ordinarily and preferably produced by a hard soap, stearic or like acid, and triethanolamine stearate or like substance. If desired the stearic acid may be omitted altogether from such a composition.

The character of the surface of the panel drawing board on which the writing occurs and the character of the crayon employed according to my invention, are interdependent. For example, the glazed surface of the panel board can be marked on by an ordinary soft lead pencil, but after such marking is made it is practically impossible to remove it easily without washing the surface. On the other hand the usual wax crayons on the market are generally too hard to be tacky and to adhere to my glazed surface in writing with the usual rapidity and pressure to make legible marks. The crayons now on the market are of a hardness to withstand changes in tem-

perature above and below ordinary room temperature, but are correspondingly too hard for suitable marking on the glazed surfaces of my invention. Varying the proportions of their ingredients may make them more tacky but they then melt too easily and are not adapted for free writing, and have not sufficient inherent strength. The glazed surface of my invention, therefore, requires a special crayon. So far as the crayon itself is concerned, it of course is adapted for writing on surfaces other than glazed surfaces. For instance, it can be used for writing on slate or porous materials, but if so used it sinks into the surface of the slate or similar hard porous material and it is practically impossible to remove it by ordinary erasing means. The same is true of paper surfaces which depend somewhat on the abrasive action of their fibers to remove particles of graphite from lead pencils or crayons applied thereto and must be erased by abrasion at least in part. My crayon, however, is intended especially to be used on my glazed surface board, and the adhesive tacky material forming these marks is such that it will adhere to the glazed surface without causing any dusting or crumbling but when a soft cotton cloth is run over it, the cloth has greater adsorption for the crayon material than the glazed surface has for the crayon material, and consequently the crayon is easily removed by gentle rubbing without abrasion.

In forming the board, as mentioned above, a suitable foundation or backing is prepared and on this a glazed surface is applied by any suitable method of application such as by brushing, spraying, dipping, flowing, rolling or printing on the surfaces may be applied as a sheet. As noted above the foundation of the board may be of pasteboard or various other materials, the foundation and coating being sufficiently stiff inherently to permit marking by crayon thereon. The size of the article may to some extent determine the method of application and this size may range from the smallest memorandum slip to that of a board such as a blackboard covering a whole wall area. The size of the article may also determine the type of finish to be applied or built up, thus a high gloss surface is not objectionable in a small telephone memorandum pad which may be easily moved about in order not to reflect light disagreeably into the writer's eyes. A high gloss on the other hand might be very objectionable if it were to replace the customary blackboard in a schoolroom, and for this purpose an egg-shell or flat finish is used and reflected light is dispersed in such a way that the schoolroom is lighter and written marks on the board are legible from all angles.

Referring now to the drawing and particularly to Fig. 1, there is shown a panel board which is made up of an underbody of cement-asbestos or wood fiber board or other suitable material, 1, on which is placed a coating of vinylite or other resin 2 containing a pigment. This board may be used with a crayon 3 composed of triethanolamine soap or similar material and pigment contrasting with the board in color. In Fig. 2 another type of panel board is shown comprising three layers, the underbody 4 of wood fiber, etc., on which is superimposed a laminated sheet of opaque white, yellow or other colored litho-paper 5. Over this is placed a coating of clear vinylite or other lacquer or a sheet of cellulose acetate or other cellophane 6. With this may be used a crayon 3 similar to that described in Fig. 1 or other type of crayon.

The following specific examples are embodied-

ments of panel drawing boards made in accordance with my invention and to be employed with the crayons, examples of which are given later herein. It is to be understood that these examples as well as the boards and crayons shown in the drawing are given simply as illustrations and the invention is not to be restricted thereto except as indicated in the appended claims.

10

## EXAMPLES OF BOARDS

## Example 1

In order to produce a panel drawing board of inexpensive construction which may be framed and employed as an easel board or similar board, white cardboard is laminated with chip board by means of cold or hot glue in the manner ordinarily used by pasteboard box manufacturers. Upon this laminated structure a viscose cellophane sheet is superimposed and cemented on the face of the white cardboard by means of a nitrocellulose lacquer or similar cementing material. The resultant product is a laminated structure consisting of cellophane over white cardboard over chip board producing an opaque or nearly opaque appearance with a glazed surface of a non-abrasive character. The surface is substantially without roughnesses, except for slight undulations, and is of sufficient stiffness to permit marking thereon with an unctuous crayon of the kind herein described. The surface may be marked on with blue or other contrasting colored crayon and the marking may then be easily erased by rubbing with a soft cloth which does not abrade the surface but simply absorbs the crayon without appreciable smearing.

Instead of the chip board I may employ wood fiber board or brown pasteboard, and instead of the cellophane sheet of viscose I may employ cellulose acetate or the vinylite type of cellophane sheet.

## Example 2

Where the foundation of the panel drawing board is to have a border design representing the margin of a finished drawing board, or where it is to be printed with the alphabet, numbers or any other desired design, I preferably use white "litho" paper on which such border or other design is printed. This is then laminated with a vinylite or other sheet on the customary machines for this purpose, using any desired cementing material. The roll of printed litho paper laminated with the vinylite sheet is then cut into any desired size by a paper cutting machine and is further laminated with a brown pasteboard back to give it the desired stiffness for marking with a hand crayon. The result is similar to that given in Example #1.

Instead of the wood fiber board, I may employ pasteboard and instead of the litho paper I may employ glazed unprinted finished paper of any color and the vinylite lacquer may be applied by dipping. In making up this form of panel drawing board the pasteboard is laminated with the paper and when the cementing material has set the laminated sheet is dipped into a vinylite solution of the proper consistency, removed, drained and allowed to dry.

70

## Example 3

Instead of the structures given in the above examples, I may employ wood fiber board as the foundation and apply on it a vinylite solution containing a white pigment such as zinc or titanium oxides. The wood fiber board is sanded

to remove protuberances, surface scratches, etc., and the vinylite solution containing pigment is then applied to this by any of the ordinary methods such as by brushing, spraying, flowing, roll-coating. Enough material is applied in one coat to give the desired smoothness or covering, or if necessary two or more coats of a thinner consistency may be applied if desired to give the glazed coating like that of Example #1, on the panel drawing board.

10

## Example 4

A panel drawing board which may be used as an easel board or which may be attached to a wall, may be made as follows:—Cement-asbestos board 15 is sanded to give a smooth surface, is sprayed with a vinylite primer solution containing a pigment and the sprayed board is then placed in a heated oven of any desired temperature, say 140° F. When dry the board is sanded again and recoated 20 with the primer solution and dried as before and resanded. A vinylite finishing solution containing white or other pigment is then applied by spraying and the drying and sanding operations repeated. A second or third coat of finishing 25 solution is then applied and dried. No further sanding operation is necessary and the resulting surface constitutes the desired glazed surface. The pigments employed may be of any desired color. For white I prefer to employ titanium 30 oxide, for blue an ultramarine blue, for red a toluidine toner, for black I may employ carbon black. Other colored pigments may, of course, be employed. Instead of drying the material after the primer coating at elevated temperatures, 35 it may be dried at ordinary temperature and coating material may be applied by other means than the spraying. The sanding operations are preferred in order to give a thoroughly smooth surface, but may be omitted if a sufficiently thick coating is applied so that the final glazed surface is 40 substantially free from roughnesses and abrasive characteristics.

This board so prepared is suitable for an easel board. It may be framed if desired. I also prefer 45 it as a wall panel. A board prepared as above may be fastened to a wall by any of the usual methods such as with an adhesive cement or by other means of direct attachment as nailing or by enclosing it in a framework attached to a wall. 50

## Example 5

Other coating materials for my panel drawing board may be employed to give the desired glazed surface than those mentioned in the preceding 55 examples. For example I have successfully employed a casein solution as a coating. The casein is prepared by adding to 1 gallon of water heated to about 158° F. 1 pound of casein. The mixture is stirred for about five minutes or until the 60 casein is fairly well swelled. 1/4 pound of borax is then added and the mixture stirred until the casein is thoroughly dispersed. Smooth white cardboard is then dipped into the casein solution, further diluted with water to give increased flow 65 if desired, removed and the excess allowed to drain off and dried at room temperature. The cardboard is preferably of sufficient inherent stiffness and with the coating of casein to permit marking thereon. One or more coats of casein 70 may be given and the casein may be used with or without pigment. The resulting surface is the desired glazed surface without abrasive characteristics suitable for marking with the unctuous crayons herein described.

75

Instead of white cardboard I may employ for example yellow cardboard suitable for bridge scores and coated with a transparent glyptal resin lacquer or varnish. The cardboard is of sufficient stiffness to permit marking thereon and the scores may be made thereon and erased repeatedly.

*Example 6*

A somewhat more expensive type of board may 10 be made of a sheet metal suitably treated. For example a piece of sheet metal such as iron or aluminum is coated by any desired method with spar varnish paint containing a pigment such as 15 chromium oxide green and when dried is given a final coat of clear bakelite, alkali- and acid-resisting varnish. It may be then air-dried or oven-dried as desired, and the surface will be found to have the desired finish.

Instead of the metal coated in this manner, I 20 may employ such sheet metal with a vitreous white opaque enamel coating such as that employed on enamelled cooking utensils or bathtubs, and applied by firing to give a glassy surface to the metal. Instead of the metal base I may 25 employ a sheet of polished glass for the panel drawing board, the glass being coated on one side with sufficient linseed oil paint, containing for example yellow pigment such as lead chromate to make the glass substantially opaque. The uncoated side 30 then provides a satisfactory glazed surface. Such a structure is relatively rigid and expensive. In place of it I may employ a molded resin such as urea-formaldehyde resin. In making up a structure 35 of this sort, as a panel drawing board, the pigment and the wood flour are incorporated in the plastic resin and the mass cast or rolled out into sheets and hardened to give the desired glazed surface. Similarly I may employ instead 40 of the molded resin, glazed pottery or porcelain for some purposes.

*Example 7*

In order to produce a panel drawing board of a 45 flexible character, but with sufficient stiffness to permit marking thereon with hand crayon, I spray-coat a heavy cotton cloth of any desired color, preferably of thick and opaque material. The spray-coat is formed of cellulose ester lacquer such as cellulose acetate or nitrocellulose lacquer 50 and a sufficient quantity is applied to make it smooth and impervious to the crayon. I prefer for this purpose to give the cloth a number of spray coats. The coat may be pigmented or not as desired. I usually prefer to add a pigment. A 55 sufficient thickness of coat is given so that the surface has the desired smooth unroughened and non-abrasive character suitable for use of the crayon herein described. After preparation of this cloth, it may be attached to a shade roller for 60 use as a roller panel board.

*Example 8*

As a toy I may employ an ordinary good grade 65 of magazine paper printed with a line-drawing picture of a bird or other animal. The paper is sprayed with a clear vinylite lacquer or varnish making it possible for a child to fill in the colors of the animal with the crayons herein described, erasing these and repeating the process at will. 70 The assembly is of sufficient stiffness so that it permits the repeated marking and erasure of the crayons herein described.

*Example 9*

The usual slate or composition wall black- 75 boards in general use may be treated to render

them satisfactory for use in accordance with my invention. For example, a natural slate blackboard fastened to a wall of a room by any of the usual means such as adhesive cement or by nailing or by enclosing in a framework attached 5 to a wall, is first cleaned with dilute hydrochloric acid or other cleansing material and the surface is rubbed down to remove the larger abrasive protuberances and sprayed with a priming coat containing a colored pigment such as yellow 10 ochre or a pigment of any color suspended in a properly plasticized vinylite solution. This spraying may be followed by one or more sprayed finishing coats with or without a pigment, the vehicle of which consists of a vinylite solution 15 properly plasticized. By this means the board is transformed into a panel drawing board having the desired glazed surface and other characteristics of my invention.

The boards may be of various colors as noted 20 in the above examples, but I prefer for general purposes light colors such as white, cream, buff and the like.

The crayons to be used with the above boards are of an unctuous type which when their writing point is applied to the glazed surface of the board will be sufficiently tacky so as to leave clearly legible marks which may be repeatedly applied and repeatedly erased without substantial staining. These crayons contain a substance 30 or substances which provide a hardening, lubricating and tacky characteristic therein, but in proportion preferably so that the crayon does not soften or harden appreciably at temperatures 35 in a range of about 15° F. above or below room temperature and so that when the crayon is applied to the surface it has about the same drag as that of a soft lead pencil when applied to the usual writing paper.

I have discovered in accordance with my invention that a crayon suitable for my purposes may be made of a solid solution of water-soluble soaps with an appropriate color added. I prefer to employ ordinary hard soap such as sodium oleate or sodium palmitate or sodium stearate, 45 or mixtures of these, dissolved in a substance of acid nature such for example as stearic acid or acid resin or gum, at slightly elevated temperature, reacted while molten with an alkaline substance such as triethanolamine and/or other 50 ethanolamine added in sufficient quantity to react with all or most of the acid material present, thus forming a triethanolamine soap with the acid substance. To the resultant mass a dry colored pigment or dye may be added or incorporated in the soap. Examples of other 55 acid materials which may be employed, are asphaltic materials, beta-naphthol tar, resins such as shellac, dammar gum, rosin, naphthenic acid, synthetic gums and resins. I prefer to have an 60 excess of stearic acid or other acid in the final product so that the product has a slightly acid reaction.

In the practice of the invention in order to obtain certain desirable physical characteristics in the finished crayon there is also a wide choice in the kind of alkaline material used to combine with acidic substances such as those mentioned above. For example the ordinary commercial grade of triethanolamine customarily contains in addition to triethanolamine approximately 5% of monoethanolamine and 17.5% diethanolamine, either of which constituents may be used alone or together to produce desirable results. The homologues of the ethanolamines, having proper- 70 75

ties similar to the ethanolamines, may be advantageously used. Instead of using the chemical derivatives which are related to the mono-hydric alcohols, substances related to the ethanolamines and similar to them but derived from the dihydric or polyhydric alcohols such as the glycols, glycerine and the like may be used. In fact various organic basic materials may be used in combination with organic acid materials to produce useful substances similar to the soaps, for example dimethyl aniline in combination with oleic acid. I have also found that a crayon for repeated marking and erasure may be made from a solid mixture of a triethanolamine soap and a coloring material.

Also, in place of a soap, I have found that it is possible to use the so-called water-soluble waxes such as the glycol stearates, dihydroxyethylamine linoleate, etc. For the soap I have also found that sulphonated oils and waxes, such as the sodium salt of sulphonated castor oil, or sulphonated tallow, and the like may be used to advantage. Also these sulphonated oils and waxes when uncombined with an alkali may be used as the acidic substance in my crayons.

In the practice of the invention it is often desirable to obtain certain physical characteristics in the crayon which can be obtained by the addition of a conditioning or tempering agent. By conditioning or tempering agent is meant an added substance which is not in itself a soap but which is added to the mixture of soaps in order to make the mixture harder or softer or which gives the crayon less or more drag, or other desired properties. It is generally possible to obtain the desired physical characteristics by changing either the acidic substance or the type of soap used but at times it is desirable to use a certain mixture of soaps which do not give the exact physical characteristics desired and the use of conditioning agents is important. These conditioning agents may be waxes in the nature of paraffin wax, beeswax, carnauba wax, halowax and the like, and mineral extenders or fillers such as blanc fixe, or soapstone and the like.

The examples of crayons given below are embodiments of the invention as I now prefer to practice it with the panel drawing boards above. It is to be understood that the invention is not to be restricted thereto except as indicated in the appended claims:—

#### EXAMPLES OF CRAYONS

##### Example 10

25 pounds of ordinary commercial hard soap flakes of either Ivory soap or Palm Olive soap, are dissolved in 22 pounds of melted stearic acid. This solution is effected in an open or closed kettle with any appropriate source of heat and the mass is agitated during dissolving. The agitation may be mechanical or by hand but it is important that the soap not be permitted to stick or burn to the bottom or sides of the kettle. When all of the soap has gone into solution and while continuing the stirring 8.8 pounds of triethanolamine are added, either at one time or slowly, together with 14 pounds of the pigment chromium oxide green prepared as follows:— In a separate, small container the chromium oxide is made into a paste with part of the triethanolamine, gradual additions of the latter being made until the pigment is thoroughly wetted and the mass has reached a fairly stiff paste consistency. Then the remainder of the

triethanolamine is added. When thoroughly mixed with the rest of the material the whole mixture is then poured into the stearic acid-soap melt and stirred until the reaction between the triethanolamine and the stearic acid is complete, a matter of two or three minutes. The stirring is then continued until substantially all of the stearic acid has been reacted upon by the triethanolamine, and triethanolamine stearate is formed and there is an even distribution of the color throughout. The mass in the kettle at this time is a molten solution of soaps in one another. The resultant colored mass is now poured into molds, or it may be permitted to cool until a desired temperature and consistency is attained to extrude it through appropriate machines into the desired shapes, or it may be cut or otherwise formed into any suitable shape by any of the methods known in the art of making marking materials.

##### Example 11

20 pounds of stearic acid is melted as in Example 10 in an appropriate kettle and 25 pounds of sodium stearate is slowly added with agitation. The agitation is continued until all of the sodium stearate is in solution. 8.8 pounds of triethanolamine preferably incorporated with 10 pounds of carbon black preferably in the same manner as indicated in Example 10 is now added and agitation is continued until all of the triethanolamine has reacted with the stearic acid and formed triethanolamine stearate. 7 pounds of paraffin wax are now added. The mixture is then molded or extruded into the form of a crayon.

##### Example 12

|                  | Pounds |
|------------------|--------|
| Stearic acid     | 22     |
| Hard soap        | 25     |
| Triethanolamine  | 8.8    |
| Ultramarine blue | 13.25  |

The stearic acid is melted at a temperature of about 220° F. the soap then added, and the heat maintained, with stirring, until the soap is dissolved. The triethanolamine is mixed as in Example 10 with 13.25 lbs. of ultramarine blue and is stirred into the mass with agitation until the triethanolamine is reacted with the stearic acid. The mixture is then molded or extruded in the form of a crayon.

##### Example 13

28.8 pounds of solid triethanolamine stearate which has been previously made by the addition of 8.8 pounds of triethanolamine to 20 pounds of molten stearic acid and permitted to solidify by cooling, is placed in a container and brought to the molten condition by the application of heat. 25 pounds of sodium stearate is now added gradually and permitted to dissolve. The dissolution is assisted by agitation and continued heating. 7 pounds of paraffin wax are now added and 10 pounds of carbon black are thoroughly incorporated into the mixture. The mixture is then molded or extruded into the form of a crayon.

The following formulae are for crayons suitable for climates where the temperature does not ordinarily exceed 75° F. or where the intended use of the crayons permits the use of a fairly large diameter stick of a minimum of at least  $\frac{1}{2}$  inches in diameter, as in school blackboard use, so that the bending character of the material is not an important factor. They are not as tough as the soap crayons and all have

a smaller softening range but otherwise possess desirable properties for marking on my panel drawing boards.

*Example 14*

|                          | Pounds |
|--------------------------|--------|
| 5 Ceresine               | 40     |
| Ultramarine blue pigment | 24     |

The ceresine is heated to about 200-210° F. When thoroughly melted the blue pigment is 10 stirred in and the mixture cooled and given a crayon shape.

*Example 15*

|                    | Pounds |
|--------------------|--------|
| 15 Ceresine        | 35     |
| Sulphonated tallow | 5      |

Chromium oxide green pigment

The binding materials, ceresine and sulphonated tallow, are heated to about 200-210° F. 20 When thoroughly melted and blended the chromium oxide is added and well stirred in, the 25 mass is cooled and shaped.

*Example 16*

|                                                   | Pounds |
|---------------------------------------------------|--------|
| 25 Paraffin wax of melting point of about 130° F. | 20     |
| Stearic acid                                      | 10     |
| Candelilla wax                                    | 10     |
| Spermaceti                                        | 1      |
| 30 Ultramarine blue                               | 23     |

The paraffin wax, stearic acid, candelilla wax and spermaceti are melted and blended together. The pigment is added and well stirred in, the 35 mass is cooled and shaped.

35 Soap-containing hand-size crayons made in accordance with the above examples have an unusual strength. They may be dropped from a height of 4 to 10 feet on hard concrete or wooden floors without causing the crayon to break even 40 when unencased. A similar drop would break a chalk or wax crayon into many small bits.

The crayons and boards described in the specific examples have the desirable characteristics mentioned. The boards are of opaque or nearly 45 opaque appearance. They have a glazed surface of a non-abrasive character substantially without roughnesses except for possible slight undulations. All of the crayons are unctuous. The soap crayons have an inherent toughness as described 50 above. They do not soften or harden appreciably at temperatures in a range of about 15° F. above or below room temperature and all 55 crayons are tacky when the point is touched on the glazed surface so that they are capable of depositing on the marking surface clearly legible marks of about the same drag as that of a soft pencil if applied to ordinary writing paper. All 60 of the crayons may be removed by simple rubbing, without appreciable smearing, with a soft cotton cloth without leaving a stain or any substantial residue of the crayon on the surface.

The expression "pasteboard" as used in the appended claims is intended to include chip board, wood fiber board, brown pasteboard and card-board.

The panel drawing boards herein described in accordance with my invention are substantially water-repellent or water-resistant. They are tough enough not to crack easily. The cellulose 70 foundation boards do not tear easily and at the same time are not so hard as to be brittle. They are reasonably resistant to the action of light, atmospheric attack and temperature changes.

I claim:

75 1. In combination, a panel drawing board

which is at least partially opaque having a glazed surface of a non-abrasive character substantially without roughnesses, except for possible slight undulations, and an unctuous crayon of contrasting color for marking thereon whose composition is of an inherent hardness if employed unencased and in the usual hand crayon size sufficient for hand marking and which does not soften or harden appreciably at temperatures in a range of about 15° F. above or below room temperature, 10 and is tacky when its marking surface is touched on said glazed surface, so that said crayon will deposit on said surface clearly legible marks with about the same drag as that of a soft lead pencil on writing paper, but may be removed by simple 15 rubbing without appreciable smearing with a soft cloth without leaving a stain or any substantial residue of said crayon on said surface.

2. In combination, a panel drawing board which is at least partially opaque comprising a 20 relatively flat underbody and a glazed surface coating thereon of a non-abrasive character substantially without roughnesses, except for possible slight undulations, and an unctuous crayon of contrasting color for marking thereon whose 25 composition is of an inherent hardness if employed unencased and in the usual hand crayon size sufficient for hand marking and which does not soften or harden appreciably at temperatures in a range of about 15° F. above or below room 30 temperature, and is tacky when its marking surface is touched on said glazed surface, so that said crayon will deposit on said surface clearly legible marks with about the same drag as that of a soft lead pencil on writing paper, but may be removed by simple rubbing without appreciable smearing with a soft cloth without leaving a stain or any substantial residue of said crayon on said surface.

3. In combination, a panel drawing board which is at least partially opaque comprising a substantially flat sheet having a lacquer coating thereon and providing a glazed surface of a non-abrasive character substantially without roughnesses, except for possible slight undulations, and an unctuous crayon of contrasting color for marking thereon whose composition is of an inherent hardness if employed unencased and in the usual hand crayon size sufficient for hand marking and which does not soften or harden appreciably at 40 temperatures in a range of about 15° F. above or below room temperature, and is tacky when its marking surface is touched on said glazed surface, so that said crayon will deposit on said surface clearly legible marks with about the same 45 drag as that of a soft lead pencil on writing paper, but may be removed by simple rubbing without appreciable smearing with a soft cloth without leaving a stain or any substantial residue of said crayon on said surface.

4. In combination, a panel drawing board which is at least partially opaque comprising a paper-containing sheet and a cellophane sheet secured upon the face of said first-mentioned sheet, and providing a glazed surface thereon of a non-abrasive character substantially without roughnesses, except for possible slight undulations, and an unctuous crayon of contrasting color for marking thereon whose composition is of an inherent hardness if employed unencased and in the usual hand crayon size sufficient for hand marking and which does not soften or harden appreciably at temperatures in a range of about 15° F. above or below room temperature, 70 and is tacky when its marking surface is touched 75

on said glazed surface, so that said crayon will deposit on said surface clearly legible marks with about the same drag as that of a soft lead pencil on writing paper, but may be removed by simple rubbing without appreciable smearing with a soft cloth without leaving a stain or any substantial residue of said crayon on said surface.

5. In combination, a panel drawing board which is at least partially opaque comprising a cement-  
10 asbestos wallboard coated with a vinylite resin solution to give a glazed surface of a non-abrasive character substantially without roughnesses, except for possible slight undulations, and an unctuous crayon of contrasting color for marking  
15 thereon whose composition is of an inherent hardness if employed unencased and in the usual hand crayon size sufficient for hand marking and which does not soften or harden appreciably at temperatures in a range of about 15° F. above or  
20 below room temperature, and is tacky when its marking surface is touched on said glazed surface, so that said crayon will deposit on said surface clearly legible marks with about the same drag as that of a soft lead pencil on writing paper, but may be removed by simple rubbing without appreciable smearing with a soft cloth without leaving a stain or any substantial residue of said crayon on said surface.

6. In combination, a panel drawing board which  
30 is at least partially opaque having a glazed surface of a non-abrasive character substantially without roughnesses, except for possible slight undulations, and an unctuous crayon of contrasting color having a hardening, lubricating and tacky mate-  
35 rial therein, substantially free from brittleness and of a hardness if employed in the usual hand crayon size sufficient for hand marking but not softening or hardening appreciably at temperatures in a range of about 15° F. above or below  
40 room temperature, and is tacky when its marking surface is touched on said glazed surface so that said crayon will deposit on said surface clearly legible marks with about the same drag as that of a soft lead pencil on writing paper, but may be  
45 removed by simple rubbing without appreciable smearing with a soft cloth without leaving a stain or any substantial residue of said crayon on said surface.

7. In combination, a panel drawing board  
50 which is at least partially opaque having a glazed surface of a non-abrasive character substantially without roughnesses, except for possible slight undulations, and an unctuous crayon of contrasting color for marking thereon whose composition  
55 is of an inherent hardness if employed unencased and in the usual hand crayon size sufficient for hand marking and which does not soften or harden appreciably at temperatures in a range of about 15° F. above or below room temperature,  
60 containing a hard soap, a triethanolamine soap and stearic acid having sufficient slipperiness to move rapidly across the surface in marking, but is tacky when its marking surface is touched on said glazed surface and will deposit thereon clearly legible marks with about the same drag as that of a soft lead pencil on writing paper, but may be removed by simple rubbing without appreciable smearing with a soft cloth without leaving a stain or any substantial residue of said  
65 crayon on said surface.

8. In combination, a panel drawing board which is at least partially opaque having a glazed surface of a non-abrasive character substantially without roughnesses, except for possible slight  
70 undulations, and an unctuous crayon of contrast-

ing color for marking thereon whose composition is of an inherent hardness if employed unencased and in the usual hand crayon size sufficient for hand marking and which does not soften or harden appreciably at temperatures in a range of  
5 about 15° F. above or below room temperature, containing a hard soap, triethanolamine soap and a wax having sufficient slipperiness to move rapidly across the surface in marking, but is tacky when its marking surface is touched on said  
10 glazed surface and will deposit thereon clearly legible marks with about the same drag as that of a soft lead pencil on writing paper, but may be removed by simple rubbing without appreciable smearing with a soft cloth without leaving  
15 a stain or any substantial residue of said crayon on said surface.

9. A panel drawing board for repeated marking and erasure, which is at least partially opaque and having a glazed surface, comprising a relatively flat foundation and a glazed coating adhering to the face of said foundation, said foundation and coating being sufficiently stiff inherently to permit marking by a crayon thereon, said surface being of a non-abrasive character  
20 substantially without roughnesses except for possible slight undulations, capable of repeated marking and erasing without substantial staining by a crayon which is tacky on said glazed surface.

10. A panel drawing board for repeated marking and erasure, which is at least partially opaque and having a glazed surface, comprising a relatively flat cellulose foundation and a glazed coating adhering to the face of said cellulose, said cellulose and coating being sufficiently stiff inherently to permit marking by a crayon thereon, said surface being of a non-abrasive character substantially without roughnesses except for possible slight undulations, capable of repeated marking and erasing without substantial staining by a crayon which is tacky on said glazed surface.

11. A panel drawing board for repeated marking and erasure, which is at least partially opaque and having a glazed surface, comprising a relatively flat sheet of cellulose and a glazed coating adhering to the face of said cellulose, said cellulose and coating being sufficiently stiff inherently to permit marking by a crayon thereon, said surface being of a non-abrasive character substantially without roughnesses except for possible slight undulations, capable of repeated marking and erasing without substantial staining by a crayon which is tacky on said glazed surface.

12. A panel drawing board for repeated marking and erasure, which is at least partially opaque and having a glazed surface, comprising a sheet of pasteboard and a glazed coating on the face of said pasteboard, said surface being of a non-abrasive character substantially without roughnesses except for possible slight undulations, capable of repeated marking and erasing without substantial staining by a crayon which is tacky on said glazed surface.

13. A panel for writing, drawing and the like, having a board containing an organic resin plastic composition of a character to display clearly marks made thereon and of sufficient rigidity to resist scarring by pressure in marking thereon.

14. A panel for writing, drawing and the like, having a board containing an organic cellulose plastic composition of a character to display clearly marks made thereon and of sufficient rigidity to resist scarring by pressure in marking thereon.

15. A panel for writing, drawing and the like, having a board containing an organic casein plastic composition of a character to display clearly marks made thereon and of sufficient rigidity to resist scarring by pressure in marking thereon.
16. A panel for writing, drawing and the like, having a board containing an organic plastic composition of a character to display clearly marks made thereon and of sufficient rigidity to resist scarring by pressure in marking thereon.
17. In combination a panel for writing, drawing and the like, having a board with a glazed surface which has the characteristics of a molded resin, and an unctuous crayon of contrasting color for marking thereon whose composition is of an inherent hardness if employed uncased and in the usual hand crayon size sufficient for hand

marking and which does not soften or harden appreciably at temperatures in a range of about 15° F. above or below room temperature, and is tacky when its marking surface is touched on said glazed surface, so that said crayon will deposit on said surface clearly legible marks with about the same drag as that of a soft lead pencil on writing paper, but may be removed by simple rubbing without appreciable smearing with a soft cloth without leaving a stain or any substantial residue of said crayon on said surface.

18. In combination a panel for writing, drawing and the like, having a board with a surface which has the characteristics of a molded resin, and an unctuous crayon which comprises the combination of a soap, a fatty acid, ethanolamine and coloring material.

CHARLES B. CHATFIELD.